

1,050,406.

S. VEIT.  
PAPER MAKER'S DRYING FELT.  
APPLICATION FILED SEPT. 16, 1908.

Patented Jan. 14, 1913.



Witnesses:

*O.O. Kedebbrand*

*N. Strauss*

By

*Sigmund Veit,*  
*Max L. Mifflin*  
Inventor:  
his Attorney.

# UNITED STATES PATENT OFFICE.

SIGMUND VEIT, OF GÖPPINGEN, GERMANY.

## PAPER-MAKER'S DRYING-FELT.

1,050,406.

Specification of Letters Patent. Patented Jan. 14, 1913.

Application filed September 16, 1909. Serial No. 518,032.

*To all whom it may concern:*

Be it known that I, SIGMUND VEIT, citizen of the German Empire, residing at Göppingen, in the Kingdom of Wurttemberg, Germany, have invented certain new and useful Improvements in Paper-Makers' Drying-Felts; and I do hereby declare the following to be a full, clear, and exact description of the invention, such as will enable others skilled in the art to which it appertains to make and use the same.

This invention relates to drying felts used in the paper makers' art, such felts serving to feed the paper sheet forward during the process of manufacture and at the same time to press the same against the surface of the heated drying cylinders for the purpose of drying the same. In order to carry out this step of the process in an efficient manner it is aimed to provide felts which give to the paper the desired translucency and smooth appearance and leave no imprint upon the same, and which, at the same time, will not become clogged and foul.

The felts hitherto employed were woven either entirely of wool, entirely of cotton, or of half-wool, that is to say, wool and cotton fiber spun together. The felts made or woven entirely of wool possess the advantage of readily undergoing the operation of fulling, whereby a compact felted surface may be imparted to them, which is very favorable to the quality and the translucency of the paper produced when employing such felts. Moreover, the absorptive action of such felts and hence their drying properties are very great. The seam of such felts having been obliterated by the fulling process, no danger of marking the paper is to be feared. However, these woolen felts absorb too much moisture and dry very slowly. Hence the speed of working is materially diminished and it often occurs that these felts become injuriously clogged and foul. This is a serious disadvantage in the case of rapid paper machines. In order to avoid this drawback, cotton felts have been proposed and frequently employed. But these felts, not being susceptible of fulling, their texture is open and is impressed on the paper. The seam is also so impressed. Only an inferior quality of paper can be made with their aid under these circumstances and for the further reason that such felts are stiff and unelastic. While felts made of half-woolen threads have been proposed to over-

come the above objections, they have not been found to do so to any material extent and, indeed, they have for this reason found only a very restricted use in this art. 60

It is the object of this invention to effectively avoid the above objections and to combine all the desirable qualities of a felt appearing from the above.

For this purpose my invention consists 65 in a felt made in two layers, one layer being made of animal fiber such as wool, while the other layer is made of vegetable fiber, such as cotton mixed with animal fiber such as wool. The amount of animal 70 fiber added to the vegetable or cotton fiber is preferably from 10 to 20 per cent. The thread or yarn from which the mixed cotton and wool layer is made or woven may be made by adding wool threads to the cotton threads in forming the yarn, or by adding wool to the cotton in spinning the 75 yarn, or by spinning half wool instead of cotton. The layer of animal fiber is the one designed to come into contact with the 80 paper during the feeding and drying operation. The two layers are united in any suitable manner, for example by a binding warp thread similar to those employed in making piled fabrics. Said binding warp 85 thread should be of animal fiber or wool or of half-wool, that is, of wool mixed with cotton.

In the accompanying drawing is represented diagrammatically the structure of a 90 drying felt made according to this invention.

In this drawing Figure 1 represents a section transverse to the weft threads of such a fabric, and Fig. 2 a similar section on a plane at right angles to the plane of Fig. 1. 95

The weft threads of the upper woolen or animal fiber layer of the felt are represented at *a*, while those of the lower mixed 100 layer are shown at *b*. The connecting warp layer is represented at *c*.

The drying felt so made is then thoroughly fulled, whereby the entire fabric is thoroughly 105 felted on the surface and, in case these binding threads are of wool or half wool, the said binding threads are also thoroughly fulled. The seams of the fabric are also thereby felted over and obliterated, so that the felt will not produce any design or 110 crease on the paper web for which the same is employed.

The drying felt thus described combines the valuable properties of an all-wool felt with those of an all-cotton felt. By virtue of the upper layer of animal fiber it has 5 the smoothness, elasticity and absorbent qualities of the former while the lower layer of mixed vegetable and animal fiber imparts to the same the quick drying action of the latter and thereby preserves it from 10 decomposition and from choking up.

In some cases the drying felt thus made may be employed with the layer containing 15 the vegetable fiber in contact with the paper, since this layer can be well fulled by reason of the wool contained therein, and its seam will leave no mark or impression.

This new drying felt combines great advantages for the art of paper making in 20 which rapid work is of importance with comparative economy.

The rapid work is promoted by the absorptive properties of the same while the fact that it lasts much longer and is cheaper 25 to manufacture than woolen felts results in a very material economy.

What I claim and desire to secure by Letters Patent is:—

1. A drying felt for paper making con-

sisting of a layer of mixed animal and vegetable fiber, combined with a layer of 30 animal fiber, the said drying felt being fulled and felted.

2. A drying felt for paper making consisting of a layer of cotton mixed with wool, combined with a layer of wool and a warp 35 thread containing animal fiber connecting the two layers, the said drying felt being fulled and felted.

3. A drying felt for paper making consisting of a layer of mixed animal and vegetable fiber combined with a layer of animal 40 fiber, the said drying felt being fulled, and felted on, substantially its surface only.

4. A drying felt for paper making consisting of a layer of cotton mixed with wool 45 combined with a layer of wool, and a warp thread containing animal fiber connecting the two layers, the said drying felt being fulled, and felted on, substantially its surface only.

In testimony whereof I hereunto affix my signature in the presence of two witnesses.

SIGMUND VEIT.

Witnesses:

LOUIS MUELLER,  
MATHALDE K. HELD.